

W. H. MILSPAUGH,  
PROCESS OF TREATING, MOLDING, AND CASTING METALS.  
APPLICATION FILED AUG. 17, 1916.

1,279,399.

Patented Sept. 17, 1918.



INVENTOR  
William H. Millspaugh  
BY  
E. M. Marshall  
ATTORNEY

# UNITED STATES PATENT OFFICE.

WILLIAM H. MILLSPAUGH, OF SANDUSKY, OHIO, ASSIGNOR TO SANDUSKY FOUNDRY & MACHINE COMPANY, OF SANDUSKY, OHIO, A CORPORATION OF OHIO.

## PROCESS OF TREATING, MOLDING, AND CASTING METALS.

1,279,399.

Specification of Letters Patent. Patented Sept. 17, 1918.

Application filed August 17, 1916. Serial No. 115,366.

*To all whom it may concern:*

Be it known that I, WILLIAM H. MILLSPAUGH, a citizen of the United States of America, and a resident of Sandusky, county 5 of Erie, and State of Ohio, have invented certain new and useful Improvements in Processes of Treating, Molding, and Casting Metals, of which the following is a specification, reference being had to the accompanying drawings, forming a part thereof.

My invention relates to the casting of metals, and particularly to such processes as involve the pouring of the molten metal into a rotating mold.

One object of my invention is to provide a relatively simple and improved process of the aforesaid character by which a superior casting such as is capable of withstanding very high internal pressures and suitable for 20 gun barrels and the like, may be produced.

Other objects and advantages of my invention will be set forth hereinafter, and in order that my invention may be thoroughly understood, I will now proceed to describe 25 the same in the following specification and then point out the novel features thereof in appended claims.

Referring to the drawings:

Figure 1 is a sectional elevation of one 30 form of apparatus which is adapted for practising my invention.

Fig. 2 is a transverse sectional view, taken on the line 2-2 of Fig. 1.

I am aware that centrifugal casting, that 35 is, casting molten metal into rotating molds, is well known, and it has been proposed to interiorly cool the metal by introducing air. This method is, however, objectionable because of the fact that the molten metal is 40 oxidized with great rapidity and with the result that the whole interior of the casting is poor and a large amount must be cut away. Furthermore, if a sufficient blast of air is utilized before the metal is set, to 45 accomplish any useful cooling, it tends to force the molten metal toward one end of the mold, following the direction of the current of air.

According to my present invention, I pour 50 the molten metal such as steel, into a hollow cylindrical rotating mold and permit the metal to cool slightly before proceeding with the subsequent treatment. The next step in the process consists in introducing water 55 in the form of spray or steam for the pur-

pose of chilling the interior surface and forming a crust. Finally, the introduction of water is discontinued and a powerful blast of air directed through the hollow casting in process of formation. This blast 60 of air is continued until the casting is completely cooled and set.

In the drawings which illustrate suitable apparatus for performing the process as outlined above, 10 represents a cylindrical mold 65 having end flanges 11 and 12, and rings 13 and 14 by which it is rotatively mounted on rollers 15 in a well known manner.

Within the mold 10 is a metal lining 16 having a flange 17 at one end. An annular 70 stop plate 18 is adjustably mounted within the lining 16 and determines the length of the casting, the opposite end being determined by an end plate 19 which is secured to the flange 11 by bolts 20, or otherwise 75 affixed to the mold.

A pulley 21 is bolted to the flange 12 at the opposite end of the mold and constitutes a suitable means by which the machine may be driven. Instead of belting the machine 80 however, it may be connected to a driving shaft by gears or in any suitable way.

A tube or pipe 22 is supported on a stationary bracket 23 and is adapted to be adjusted to extend through the mold and into 85 a guide bracket 24 at the opposite end, as shown in broken lines in Fig. 1. The guide bracket may be swung out of the way when not in use, as shown in full lines in Fig. 1. The pipe 22 is provided with perforations 90 25 and is connected by a flexible hose or pipe 26 to any suitable source of water or other non-oxidizing cooling fluid. In addition to the liquid cooling pipe or distributer, an air pipe 27 is provided, conveniently at the same 95 end of the mold. This pipe is pivoted at 28 so that it may be swung to one side when not in use and not interfere with the water pipe.

29 designates a pouring funnel or spout 100 mounted on a truck 30 which is adapted to extend through an opening 33 in the end plate 19 and hence is adapted to discharge the molten metal, which it carries, into the mold.

Between the stop plate 18 and the end plate 19 the usual sand lining 34 is provided in the particular form of apparatus which is illustrated in the drawings.

The process will be understood from the 110

foregoing and may be described with reference to the apparatus as follows:—The mold 10 is first rotated by connecting a suitable driving shaft (not shown) to the pulley 21. 5 The molten metal is next introduced by moving the spout 29 into the position shown in Fig. 1 and pouring molten metal therein which is discharged therefrom into the mold. The metal will, on account of the centrifugal 10 action due to the rotation of the mold, conform to the inner surface of the mold of whatever shape it may be and assume a cylindrical interior curvature. 15 After a predetermined lapse of time sufficient to permit the casting to cool slightly, the pipe 22 is moved from the position shown in full lines to the position shown in dotted lines in Fig. 1, and water, steam or other 20 non-oxidized fluid is discharged from the perforations 25, into the mold. The effect of cooling fluid discharged in this manner is to chill the metal and form a crust on the surface. This crust prevents the oxidization 25 of the surface during the last step of the process which is accomplished by withdrawing the pipe 22, swinging the pipe 27 to the position shown in full lines, and turning on a blast of air which will rush through the center of the mold and carry out at the opposite end, the hot gases, etc., and continue 30 the cooling process. The air blast is maintained until the casting is completed when the mold is stopped and the casting removed. 35 The process of my present invention is commercially practicable and constitutes the solution of a well known problem which

hitherto has been approached in various ways without success. Castings by my process may be produced readily, which are particularly adapted for pipes, gun barrels, and such other structures as are called upon to resist very high internal pressures. 40

This application is a continuation in part of my application Serial No. 671,456, filed 45 January 16, 1912.

What I claim is:

1. The process of treating metal which consists in pouring the molten metal into a rapidly rotating mold and subjecting it to 50 the action of centrifugal force, then introducing a cooling fluid into the interior of the mold to chill the exposed inner surface of the metal, and introducing a blast of cooling air. 55

2. The process of treating metal which consists in pouring the molten metal into a rapidly rotating mold and subjecting it to the action of centrifugal force, then introducing a cooling liquid into the interior of 60 the mold to chill the exposed inner surface of the metal, and finally introducing a blast of cooling air until the casting is completed. 65

3. The process of casting steel which consists in pouring the molten metal into a rapidly rotating mold and subjecting it to the action of centrifugal force, allowing it to cool slightly, then spraying the interior exposed surface of the casting with water to 70 form a crust, and finally blowing cooling air through the hollow casting from end to end. 75

In witness whereof, I have hereunto set my hand this 14th day of August, 1916.

WILLIAM H. MILLSPAUGH.